

Patented Nov. 5, 1929

## UNITED STATES PATENT OFFICE

JOSEPH R. COOLIDGE, 3D, OF BROOKLINE, MASSACHUSETTS, ASSIGNOR TO MONTAN,  
INC., OF BOSTON, MASSACHUSETTS, A CORPORATION OF MASSACHUSETTS

## FIREPROOFED WOOD AND PROCESS OF TREATING WOOD

No Drawing.

Application filed December 18, 1926. Serial No. 155,768.

This invention relates to the treatment of wood to render it highly resistant to combustion. The invention involves both a novel process and also a new product.

5 The natural inflammability of wood is a very serious objection to its use for many purposes, as for example, for interior finish or for flooring in modern buildings of the fireproof type. In fact, the authorities in 10 many cities where every effort is being made to reduce the fire hazard have adopted very strict regulations as to the fireproof properties of flooring used in such buildings.

The most successful methods so far devised of treating wood to render it fireproof consists in impregnating the wood with certain water soluble salts, ammonium chloride, ammonium sulphate, borax, and the like, being commonly used for this purpose. These 20 treatments, while effective from the fireproofing standpoint, are objectionable in certain other respects. For example, an especially serious objection is the fact that the salts absorb moisture from the atmosphere in 25 damp weather, notwithstanding the presence of finish coatings of varnish, shellac, or the like, and the solution resulting from such absorption sometimes attacks the finish, and in any event leaves discolored spots or streaks 30 on the floor or finish which are highly objectionable from a standpoint of appearance. If water stands on such a floor for any length of time, as for example, water leaking from a 35 radiator, or rain driving in through an open window, the action on the salts with which the wood is impregnated is even more pronounced. Furthermore, when woods fireproofed with salts are used in locations such as cellars, basements, or the like, where, while 40 not exposed to the weather, they are, nevertheless, exposed to considerable dampness, they gradually lose their salts due to the action of the moisture. Consequently, the degree of fire protection afforded by this treatment is not permanently retained but gradually 45 is reduced.

The present invention deals with the problems presented by these conditions, and it aims to devise a method of fireproofing wood 50 which will overcome the objections above de-

scribed. It is also an important object of this invention to produce a wood fireproofed to such a degree as to meet the very severe requirements of authorities such as the underwriters' laboratories, while at the same time 55 protecting the fireproofing material from atmospheric action, and holding said material more effectively in the wood than has been possible heretofore.

According to this invention the wood is 60 impregnated with fireproofing materials of any suitable character, and a protective agent is associated with the material which prevents the deleterious action above described.

According to the preferred process the 65 wood is first impregnated with a suitable fireproofing material, such as ammonium salts, borax, and the like, such material being hereinafter referred to as "salts." I have obtained particularly satisfactory results by 70 mixing ammonium chloride and borax in equal parts, and then dissolving one part, by weight, of this mixture of salts in two parts, by weight, of water. The impregnation with these fireproofing salts may be performed 75 in any convenient manner, this part of the process being well known in this art. Assuming, for example, that the wood under treatment is red oak, an entirely satisfactory 80 impregnation can be obtained by immersing the wood in the salt solution and maintaining a pressure of approximately 200 lbs. per square inch on the solution for one hour, the solution being held at a fairly high temperature, as for example, 190° F. A pressure 85 cylinder of the type used in impregnating wood is required for this purpose. At the end of the period of one hour just mentioned it is preferable to cut off the steam and then to circulate cold water through the steam 90 heating coils in the cylinder. This operation should be continued for about an hour, the cooling of the solution precipitating the salts in the wood. As above stated, however, the impregnation of the wood with fireproofing 95 salts may be accomplished in any suitable manner, and the procedure adopted necessarily will depend somewhat upon the equipment available, the size of the pieces, the kind of wood being treated, and the like. 100

If the impregnation is performed at high temperatures, there is considerable tendency to darken the wood, but this discoloration can be reduced or entirely avoided by reducing the temperatures at which the impregnation with the salts is performed. A high temperature followed by cooling, as above described, is, however, a convenient method of introducing a high concentration of salts in the wood.

A certain amount of the water should next be removed from the wood in order to make room for the material which is to seal the salts in the wood. This may be accomplished either by subjecting the wood to a vacuum while it still remains in the treating cylinder, or the wood may be removed and partially dried. Assuming that the wood under treatment is red oak, the weight of the wood is approximately doubled by the treatment above described, about two-thirds of this increase in weight being water and one-third salt. It is preferable to reduce this water content at least 15% before proceeding with the next step of the process. Whether this is done by air or kiln drying, or by subjecting the wood to a vacuum while still in the cylinder, will depend largely upon conditions obtaining at the treating plant.

The discovery of a suitable material for holding the salts in the wood and protecting them from the action of external moisture, without at the same time decreasing the fireproofing properties of the final product, has proved to be a very difficult matter. After a long series of experiments, however, I have found that ordinary soap satisfies these requirements. Accordingly, the next step in this process preferably consists in impregnating the wood which has now been treated with fireproofing salts and then partially dried, with a solution of, say, one part of soap in five parts of water. The impregnation should be performed in a pressure cylinder, the solution being maintained at, say, 150° F. and forced into the wood under approximately 200 lbs. of pressure for a period of one hour. The wood then is removed from the cylinder and stacked when it can drain and dry out.

When the wood has dried it has an appearance substantially like untreated wood and is entirely devoid of the discolored surface which is a characteristic of wood fireproofed by the usual processes. This surface takes the ordinary finishes, such as varnish, waxes, or the like, entirely satisfactorily. I have had no difficulty in treating wood by this process so that it successfully passed the tests prescribed by the underwriters' laboratories. An important advantage of wood fireproofed in this manner as distinguished from that treated by prior processes is that it retains its fireproof characteristics indefinitely, whereas wood treated by the common commercial proc-

esses gradually loses its fireproof characteristics under many conditions of use.

While the action which takes place in the wood is somewhat obscure, it seems clear that the impregnation with the fireproofing salts results in the deposit of these salts on and in the walls of the pores and tracheids of the wood. The subsequent impregnation with soap results in coating the walls with this material, some of the soap solution probably also entering the cell walls. This coating thereafter protects the salts from the action of external moisture under ordinary conditions. The presence of the salts has the apparent effect of reducing the solubility of the soap so that the soap in the treated wood is not readily acted upon by water. The soap appears to be partly converted into the insoluble variety due to the presence of impurities in the borax. In any event, the soap assumes a rubbery consistency and becomes relatively insoluble, acting much as it does in sea water or in a strong brine.

While the foregoing is the best explanation of the favorable results obtained which I am able at this time to give, it will be understood that the invention is not limited to the theory above set forth.

As above stated, I have obtained very satisfactory results by using ordinary hard laundry soap of the tallow or tallow and resin variety. The fireproofing properties of the soap may, however, be further increased by adding to the soap solution a small proportion, say 25% of the weight of the soap, of some material such as paradichlorbenzene. The soap impregnation, particularly when a small proportion of paradichlorbenzene is used with it, has considerable merit as a fireproofing agent, although it does not afford the same degree of protection as the treatment above described.

As a further variation of this method, I may use some material, such as calcium chloride, aluminum sulphate, or the like, either with or without other salts, in effecting the first impregnation, the salts mentioned combining with the soap to form in the wood an insoluble soap that will act as a sealing agent. In fact, some action of this character appears to take place in the process above described. Also, the entire body of soap may be formed in the wood by ingredients forced into the wood in successive impregnations. While, therefore, I prefer to use the method described in detail above, it will be evident that the method is susceptible of considerable variation without departing from the essential features thereof. In fact, for many purposes it is not necessary to impart to the wood the degree of fire protection afforded by the treatment above described, and in such cases the treatment may be suitably modified.

This application and my pending applica- 130

tion Serial No. 181,276, filed April 5, 1927, have certain features in common, and the claims on the common subject matter are presented in the latter application. The claims 5 in this application are confined to features which are not claimed in the later application just mentioned.

Having thus described my invention, what I desire to claim as new is:

- 10 1. An article of the character described, comprising wood impregnated with fireproofing salts, and also impregnated for a substantial depth with soap.
- 15 2. An article of the character described, comprising wood, the walls of the pores and tracheids of which carry a water soluble fireproofing salt, and a coating of soap on said walls.
- 20 3. That improvement in processes of fireproofing wood, which consists in impregnating the wood with water soluble fireproofing salts, and subsequently impregnating the wood with a soap.
- 25 4. That improvement in processes of fireproofing wood, which consists in impregnating the wood with water soluble fireproofing salts, subjecting the wood to a drying operation, and then impregnating the wood for a substantial depth with a water solution of 30 a soap.
- 35 5. An article of the character described comprising wood impregnated with a fireproofing salt and also impregnated for a substantial depth with an insoluble metallic soap which serves as a protective agent for said fireproofing salt.
- 40 6. An article of the character described comprising wood, the walls of the pores and tracheids of which for a substantial depth carry a water soluble fireproofing salt, and an insoluble metallic soap in said pores and tracheids serving to protect said salt.
- 45 7. That improvement in processes of fireproofing wood which consists in forcing into the pores and tracheids of the wood for a substantial depth a water solution of a fireproofing salt, including in said solution a metallic salt adapted to react with a soluble soap to form an insoluble soap, and subsequently impregnating the wood so treated 50 with a solution of soap to combine in the wood with said metallic salt to produce an insoluble soap capable of sealing said fireproofing salts in the wood.

JOSEPH R. COOLIDGE, III.